

2,815,368

## COMPLEX ESTER SYNTHETIC LUBRICANTS

Alfred H. Matuszak, Westfield, N. J., assignor to Esso Research and Engineering Company, a corporation of Delaware

No Drawing. Application March 17, 1954,  
Serial No. 416,941

2 Claims. (Cl. 260—484)

This invention relates to synthetic lubricating compositions. Particularly the invention relates to new and useful synthetic lubricants that have outstanding utility at both high and low temperatures and that have, in addition, low carbonization characteristics and result in little or no sludge formation when used in automotive engines. More particularly, the instant invention relates to new and useful synthetic lubricating compositions which comprise the complex reaction products of mercapto or hydroxy acids, aliphatic carboxylic acids and organic hydroxyl containing materials.

In recent efforts to obtain superior lubricating compositions which have unusual and specific properties, there have been developed entirely new synthetic materials. In general, these new synthetic lubricants are characterized by viscosity properties that are outstanding at both high and low temperatures, especially when compared to mineral oils. These outstanding low and high temperature properties are especially desirable for use in equipment designed to operate over a great temperature differential, such as jet engines for aircraft use, combustion engines for aircraft and the like. It has been found that mineral lubricating oils are generally undesirable for the lubrication of these engines because of their high and low temperature viscosity limitations.

It has also been found that synthetic lubricants may be desirable for the lubricating of standard automotive engines. In addition to the versatility of their viscosities, the use of some types of the synthetic lubricants investigated have been found to result in very low rates of combustion chamber deposit formation, particularly when used for long periods of time. These combustion chamber deposits usually occur in the form of carbonaceous deposits on the combustion chamber surfaces. Low rates of formation of combustion chamber deposits result in increased power factor from fuel, less increase in the octane requirement of the engine, less pre-ignition tendency, and a general overall improvement in engine operation. These new and improved lubricants may also serve to reduce, or remove, the combustion chamber deposits of engines already heavily loaded with such deposits.

It has been found that for use in reciprocating engines, particularly as a lubricant for automotive engines, a lubricating composition must meet several requirements. In order to form an effective lubricating film and to maintain that film at low and high temperatures, it must have certain viscosity characteristics. At low temperatures, the lubricant must be sufficiently labile to flow through the circulatory system of the equipment and allow movement of lubricated surfaces without undue power requirement. A lubricant having an ASTM pour point below about +35° F. has sufficient low temperature lability to make it satisfactory in these respects for general use. At high temperatures a lubricant must have sufficient "body" or "thickness" to furnish and maintain a satisfactory lubricating film. It has been found that a lubri-

cant that is satisfactory in this respect will have a viscosity at 210° F. of between about 2 and 60 centistokes or 32.8 and 280 Saybolt Seconds Universal. To prevent undue lubricant loss, due to volatility and general molecular disintegration, and to insure against explosion hazards at high temperatures sometimes encountered, a lubricating composition should have a flash point in excess of about 300° F. These requisites are inherent in the term "lubricating compositions," as used in this specification, and the materials of the invention are limited to those within these operable ranges. In general, the preferred materials, as contemplated herein and as described in the preferred embodiment hereof, will have an ASTM pour point below about -15° F., a flash point above about 375° F., and will have viscosities within the range of 2.6 to 15 centistokes, or 35 to 78 Saybolt Seconds Universal at 210° F.

It has now been found, and forms the object of this invention, that the viscosity requirements as outlined above for synthetic lubricants may be met by materials which may be described as complex esters in which the portion of the ester between the terminal groups comprises a combination of varying proportions of at least one mol of either hydroxy- or mercapto-acid with a combining portion of a glycol and/or a dibasic acid.

The materials that are utilized as starting materials for the complex esters of this invention are as follows:

(1) Monohydric alcohols or mercaptans represented by the formula



wherein X is oxygen or sulfur and wherein R is an alkyl group containing from 1 to 20 carbon atoms.

(2) Aliphatic dibasic acids of the formula



wherein x is a whole number, preferably from 2 to 8.

(3) Dibasic acids of the formula



wherein y is a whole number, preferably from 1 to 8, and X is either oxygen or sulfur.

(4) Glycols of the formula



wherein n is a small whole number, preferably 2 to 5 and wherein y is a number, preferably from 1 to 20.

(5) Monobasic acids of the formula



wherein R is an organic group containing from 1 to 20 carbon atoms, preferably an alkyl radical.

(6) Mercapto- or hydroxy-acids of the formula



wherein R is hydrogen or an alkyl group containing from 1 to 10 carbon atoms, X is oxygen or sulfur, and wherein z is a whole number, preferably 0 to 12.

Using these starting materials it is possible to build compositions having the desired lubricating characteristics. Some of the preferred types of contemplated complex esters are depicted by the formulas below:

Type

1—Alcohol-hydroxy acid-dibasic acid-hydroxy acid-alcohol

2—acid-hydroxy acid-glycol-hydroxy acid-acid

3—acid-hydroxy acid-glycol-dibasic acid-alcohol

4—acid-glycol-hydroxy acid-dibasic acid-alcohol

5—alcohol-dibasic acid-hydroxy acid-glycol-dibasic acid-alcohol

6—alcohol-dibasic acid-hydroxy acid-glycol-hydroxy acid-dibasic acid-alcohol

- 7—alcohol-hydroxy acid-dibasic acid-glycol-hydroxy acid-dibasic acid-alcohol  
 8—alcohol-dibasic acid-hydroxy acid-glycol-hydroxy acid-acid  
 9—alcohol-hydroxy acid-dibasic acid-glycol-dibasic acid-hydroxy acid-alcohol  
 10—alcohol-hydroxy acid-dibasic acid-glycol-dibasic acid-alcohol

In the above types of complex esters "mercaptan" may be used instead of "alcohol" and "mercapto-acid" may be substituted for "hydroxy-acid."

It has been found that complex esters having proper lubricating characteristics will contain a total of from about 20 to 130 carbon atoms per molecule, with from 25 to 100 carbon atoms per molecule being especially satisfactory.

A partial list of the aliphatic alcohols operable in the preparation of the complex esters of this invention will include the following alcohols: methyl, ethyl, propyl, isopropyl, n-butyl, iso-butyl, sec-butyl, tert-butyl, n-amyl, iso-amyl, n-hexyl, iso-hexyl, 2-ethyl-1-butyl, 2-ethyl-1-hexyl, octyl, iso-octyl, 2-octyl, iso-nonyl, decyl, lauryl, tetradecyl, pentadecyl, octadecyl, allyl, crotyl, oleyl, the terpineols, the  $C_2$  to  $C_{20}$  Oxo alcohols, alcohols derived from the "Synol" process, those derived from the oxidation of petroleum fractions, those derived from the Guerbet reaction, those derived from the hydration of olefins, those derived via the "Oxyl" synthesis, and mixtures of the above. The corresponding mercaptans may also be used. Especially preferred are those alcohols and mercaptans containing from 6 to 10 carbon atoms.

Particularly desirable alcohols for use in this invention are those highly branched chain aliphatic alcohols prepared by the "Oxo" synthesis. The "Oxo" synthesis may be described as being the catalytic reaction of an olefin with carbon monoxide and hydrogen. The reaction occurs at temperatures in the order of 300°-400° F., at pressures in the range of about 1000 to 3000 p. s. i., in the presence of a suitable catalyst, ordinarily a heavy metal carbonyl such as cobalt carbonyl. The resulting aldehyde is subsequently hydrogenated to a primary alcohol. This process is described in U. S. Patent No. 2,327,066 issued to Roelen in 1943.

It has been found that particularly desirable alcohols for the formation of the complex esters of this invention can be prepared by the application of the Oxo synthesis to polymers and copolymers of  $C_3$  and  $C_4$  monoolefins. These monoolefins are readily available in petroleum refinery streams, and processes for their conversion to liquid copolymers have been worked out by the art. One such process, known as U. O. P. polymerization, consists of passing the olefin-containing stream in liquid phase in contact with an acid catalyst comprising phosphoric acid impregnated on kieselguhr. Other acidic catalysts, such as phosphoric acid or copper phosphate impregnated on silica gel, sulfuric acid, Friedel-Crafts catalysts, activated clays, silica-alumina, copper pyrophosphate, etc., may be used. Suitable conditions when employing phosphoric acid catalysts of the U. O. P. type are temperatures of 300° F. to 500° F., pressures from 250 to 5,000 p. s. i. and feed stocks comprising refinery streams containing propylene and mixed butylenes. Suitable feed stocks, for example, may contain from 15 to 60 mol percent propylene, from 0.5 to 15 mol percent butylenes, and from 0.1 to 10 mol percent isobutylene, the remaining being saturated hydrocarbons. Other suitable feed stocks are the dimer and trimer of isobutylene.

The preferred Oxo alcohols employed in this invention are those having from 8 to 20 carbon atoms derived from olefin copolymers having from 7 to 19 carbon atoms. In preparing these Oxo alcohols the desired olefin fraction is segregated from the crude olefin polymer product by fractionation.

The following table, for example, shows the structure and percent composition of  $C_8$  Oxo alcohols prepared

from a  $C_7$  olefin stream which had been fractionated from the products obtained by the phosphoric acid polymerization of refinery gas streams containing propylene and mixed n- and isobutylenes.

| Structure of $C_8$ Oxo alcohols prepared from $C_3-C_4$ copolymer heptenes                                                                      | Percent |
|-------------------------------------------------------------------------------------------------------------------------------------------------|---------|
| $\begin{array}{c} \text{C} \quad \text{C} \\   \quad   \\ \text{C}-\text{C}-\text{C}-\text{C}-\text{C}-\text{C}-\text{C}-\text{OH} \end{array}$ | 29      |
| $\begin{array}{c} \text{C} \quad \text{C} \\   \quad   \\ \text{C}-\text{C}-\text{C}-\text{C}-\text{C}-\text{C}-\text{C}-\text{OH} \end{array}$ | 25      |
| $\begin{array}{c} \text{C} \quad \text{C} \\   \quad   \\ \text{C}-\text{C}-\text{C}-\text{C}-\text{C}-\text{C}-\text{OH} \end{array}$          | 17      |
| $\begin{array}{c} \text{C} \\   \\ \text{C}-\text{C}-\text{C}-\text{C}-\text{C}-\text{C}-\text{C}-\text{OH} \\   \\ \text{C} \end{array}$       | 16      |
| $\begin{array}{c} \text{C} \\   \\ \text{C}-\text{C}-\text{C}-\text{C}-\text{C}-\text{C}-\text{C}-\text{OH} \\   \\ \text{C} \end{array}$       | 2.3     |
| $\begin{array}{c} \text{C} \\   \\ \text{C}-\text{C}-\text{C}-\text{C}-\text{C}-\text{C}-\text{OH} \\   \\ \text{C} \end{array}$                | 1.4     |
| 30 $\alpha$ -alkyl-alkanols                                                                                                                     | 4.3     |
| Others                                                                                                                                          | 5.0     |
|                                                                                                                                                 | 100.0   |

It will be noted that Oxo alcohols derived from the olefins produced by  $C_3-C_4$  polymerization are mostly methyl substituted.

Dibasic acids operable in the concept of this invention include the following: oxalic, malonic, succinic, glutaric, adipic, pimelic, suberic, azelaic, sebacic, fumaric, maleic, itaconic, citraconic, diglycolic, thiodiglycolic, thiadipropionic, dithiodiglycolic and the like. Especially preferred are those dibasic acids containing from 6 to 10 carbon atoms.

Operable glycols include: ethylene, the various diols, such as propane, butane-, pentane- and hexane-diols, the various polyalkylene glycols such as polyethylene glycols and polypropylene glycols, and the like. Especially preferred are the polyethylene glycols of the formula:



wherein  $n$  is an integer from 2 to 5 and where  $y$  is an integer of from 1 to 20.

Operable monobasic acids include the following: formic, acetic, propionic, butyric, 2-ethylbutyric, caproic, 2-ethyl hexanoic, caprylic, pelargonic, capric, lauric, myristic, oleic, stearic, methoxy-propionic, ethoxyethoxy-acetic, mono-2-ethyl hexyl adipate, mono- $C_8$ -Oxo-sebacate, acids derived from alcohols by caustic fusion, acids derived from petroleum fractions by oxidation, and mixtures of the above. Those acids containing from 4 to 10 carbon atoms are preferred.

Operable hydroxy- and mercapto-acids include the following: hydroxy-acetic (glycolic), hydroxy-butyric, hydroxy-caproic, hydroxy-caprylic, alpha-hydroxy-propionic (lactic), beta-hydroxy-propionic, hydroxy-stearic, and the corresponding mercapto acids, such as thio-glycolic, etc.

The preparation of the complex esters of this invention may be accomplished by either a one-step or a two-step technique.

It will be noted from examination of the various types of the complex esters contemplated as described above, that these esters are "terminated" or "stopped" by use of a monofunctional material, either an alcohol, mercaptan or an acid. In the two-step technique, the central

or "body" portion of the complex ester may be prepared in a first step by admixing the desired amount of the chosen reactants with a small amount of a catalyst and a water entrainer in a reaction zone. The catalyst may be any of the commonly known esterification catalysts, such as sodium acid sulfate, toluene sulfonic acid, sulfo-salicylic acid; sulfuric acid, zinc chloride, etc. The reaction temperature is maintained at about 150° to about 220° C. for from 2 to 6 hours, or until tests of the reaction mixture show that the esterification is substantially completed. In the second step, the "stopping" or "terminating" agent, either a monobasic acid or a monohydric alcohol or mercaptan is added in the correct amount. The reaction temperature is then maintained at about 200° to about 230° C. until such time that the neutralization number of the reaction product is at the desired low level.

However it may also be desired to prepare a half ester of a bifunctional material and then connect two moles of such half ester with a second bifunctional material. For example, the first step of such a procedure might be to react together molar quantities of an alcohol and a hydroxy acid in a first step and then react together two moles of such ester with a dibasic acid in a second step. Other variations available will be apparent to those skilled in the art.

Purification of the complex ester is accomplished by stripping off any unreacted ingredients, water entrainer, light ends and the like by a stripping step. Vacuum stripping may be desired in some instances. The material, stripped as above, may then be washed to remove any residual acidity with an alkaline solution, such as a sodium carbonate solution, etc. Final acidity may also be reduced to the desired level by filtration through alumina or charcoal or some similar adsorbent material.

In the one-step process, referred to above, the theoretical amount of all the desired reactants plus any excess are added to the reaction zone and the temperature maintained at about 190° to 230° C. for a period of time sufficient to obtain a product of the desired low neutralization number. The same general finishing procedures as outlined above may be used to prepare the final product, that is, a stripping step, using vacuum if desired, a washing step, and an alumina or charcoal treatment.

It may also be desired to add antioxidants to the esterification reaction or at other points in the process of preparing these complex ester synthetic lubricants. Such materials as phenothiazine have been found to aid in the preparation of more desirable lubricants.

The invention will be more clearly explained by reference to the following illustrative examples.

*Example I.—Preparation of type 5 complex ester (2-ethylhexanol-sebacic acid-glycolic acid-polyethylene glycol-sebacic acid-2-ethylhexanol)*

In this preparation a one-step procedure was employed. The following ingredients were charged to a 3-1 esterification apparatus equipped with stirrer, thermometer, reflux condenser and water trap.

|                                     | G.  |
|-------------------------------------|-----|
| Sebacic acid                        | 606 |
| Polyethylene glycol (M. wt. of 200) | 273 |
| Glycolic acid (70%)                 | 164 |
| 2-ethylhexanol                      | 390 |
| 10% excess 2-ethylhexanol           | 39  |
| Phenothiazine (0.5%)                | 6.5 |
| Heptane                             | 55  |
| NaHSO <sub>4</sub> catalyst (0.5%)  | 6.5 |

These ingredients were heated to reflux temperature and after 3 hours the temperature had gradually increased to 210° C. and 187 cc. of water had collected. The crude ester was then heat treated at 235° C. for 3 hours during which time the pressure was lowered to 10 mm. to remove the volatile constituents. After washing with

10% Na<sub>2</sub>CO<sub>3</sub> aqueous solution and alcohol, followed by two water washes, the material was filtered and then stripped to 162° C. at 8 mm. to give 1140 g. of lubricant having the following properties:

|    |                                      |        |
|----|--------------------------------------|--------|
| 5  | Viscosity, cs., @ ° F.:              |        |
|    | 210                                  | 14.05  |
|    | 100                                  | 86.7   |
|    | 0                                    | 4,350  |
|    | -40                                  | 94,400 |
| 10 | V. I.                                | 139    |
|    | Pour point, ° F.                     | -45    |
|    | Flash point, ° F.                    | 530    |
|    | Fire point, ° F.                     | 570    |
| 15 | 1 hr. SOD lead corrosion loss, mg    | 61     |
|    | SAE-SOD load test, lbs. <sup>1</sup> | 700    |

<sup>1</sup> SAE lubricant tester is run in at 50 lb. load for 2 minutes, then load is increased manually by 50 lbs. every 10 seconds until scuffing of bearing rings occurs.

*Example II.—Preparation of type I complex ester (C<sub>10</sub> Oxo alcohol-glycolic acid-sebacic acid-glycolic acid-C<sub>10</sub> Oxo alcohol)*

The following ingredients were used:

|    |                                                                              |     |
|----|------------------------------------------------------------------------------|-----|
| 25 | Sebacic acid                                                                 | 202 |
|    | Glycolic acid (70%)                                                          | 218 |
|    | C <sub>10</sub> Oxo alcohol (by oxonation and hydrogenation of tripropylene) | 316 |
|    | 10% excess C <sub>10</sub> Oxo alcohol                                       | 32  |
| 30 | Heptane                                                                      | 57  |
|    | NaHSO <sub>4</sub> catalyst (0.5%)                                           | 3.0 |

The C<sub>10</sub> Oxo glycolate was made by heating everything except the sebacic acid to 177° C. over a 1 hour period. The water collected was 100 cc. The sebacic acid was then added and the esterification continued to get 36.5 cc. more water by carrying the esterification temperature to 190° C. The material was then decanted from the catalyst sludge, washed with two 600 cc. portions of 2.5% Na<sub>2</sub>CO<sub>3</sub> solution and two 200 cc. portions of water and then stripped to 212° C. kettle temperature at 0.25 mm. pressure. The product had the following properties:

|    |                   |        |
|----|-------------------|--------|
| 45 | Kin. vis., cs.:   |        |
|    | 210° F.           | 7.32   |
|    | 100° F.           | 46.25  |
|    | 0° F.             | 2,520  |
|    | -40° F.           | 51,100 |
| 50 | V. I.             | 125    |
|    | Pour point, ° F.  | -45    |
|    | Flash point, ° F. | 510    |
|    | Fire point, ° F.  | 560    |

It is also within the concept of this invention to prepare synthetic lubricating compositions which comprise blends of the complex ester synthetic lubricants as described above with various of the additive materials used by the art to enhance special lubricating characteristics of the final blend. For instance, it is contemplated to blend with these complex esters viscosity index improvers such as polybutene, polyacrylate and polymethacrylate esters containing from 8 to 18 carbon atoms in the alcohol groups and other types. It is also contemplated to blend with these complex esters pour point depressants such as wax naphthalene condensation products, acrylate and methacrylate ester polymers, fumarate vinyl ester copolymers and the like. Other additives, such as detergent inhibitors, anti-rust agents, extreme pressure additives, oxidation inhibitors and the like are also compatible with these synthetic esters and blends containing them are contemplated.

The synthetic lubricants of this invention may also be used to compound various blends using as a blending agent other synthetic lubricants such as formals, polyalkylene ethers, dibasic acid esters, silicones, silicates, polyglycol ethers, ether-esters, etc. The complex esters of this in-

vention are also compatible with mineral oils of either naphthenic or paraffinic origin and blends with these materials are contemplated.

The complex esters of this invention may also be used as the base oils for the formation of lubricating grease compositions. Greases from these esters may be prepared by thickening them with any of the commonly used grease-forming soaps, such as the alkali or alkaline earth metal soaps of high molecular weight fatty acids. Soaps such as the oleates, stearates, or hydroxy stearates of sodium, potassium, lithium, calcium, barium, strontium and the like may be used. Soaps formed by heating animal, fish or vegetable oils with derivatives of the metals above may also be used.

To summarize briefly, the instant invention relates to new and improved synthetic lubricants of the complex ester type. These complex esters contain from 20 to 130 carbon atoms per molecule and are prepared by reacting a hydroxy or mercapto acid with a monofunctional and a difunctional compound selected from the following classes of materials: monobasic acids, monohydric alcohols, mercaptans, glycols, and polybasic acids. The molecule will ordinarily be terminated by a monofunctional material, usually an alcohol, a mercaptan, or a monobasic acid and will contain at least one molecule of a hydroxy- or mercapto-acid. The complex esters of the invention are preferably those having viscosities at 210° F. within the range of from 2.6 to 15 centistokes, ASTM pour points below about 35° F., and flash points above about 300° F. Especially preferred and contemplated in the preferred embodiment hereof are those complex esters having the formula



wherein R, R<sub>2</sub>, and R<sub>4</sub> are alkyl groups containing from 1 to 20 carbon atoms, preferably 6 to 12 carbon atoms, wherein X is oxygen or sulfur, wherein z is a number from 0 to 12, preferably 4 to 6, R<sub>1</sub> and R<sub>3</sub> may be hydrogen or alkyl groups of from 1 to 6 carbon atoms and



wherein R, R<sub>2</sub>, R<sub>3</sub>, R<sub>4</sub>, and R<sub>5</sub> are alkyl or alkylene groups containing from 1 to 20 carbon atoms, preferably from 6 to 12 carbon atoms, wherein R<sub>1</sub> is selected from the group consisting of hydrogen or alkyl radicals containing from 1 to 10 carbon atoms, wherein X is oxygen or sulfur and wherein z is a number from 0 to 12, preferably 4 to 6.

What is claimed is:

1. A synthetic lubricating composition having an ASTM pour point below about -15° F., a flash point above about 375° F., and a viscosity at 210° F. between about 2.6 and 15 centistokes, which comprises a material of the formula:



wherein R and R<sub>2</sub> are alkyl groups containing from 6 to 10 carbon atoms, wherein X is selected from the group consisting of oxygen and sulfur, wherein x is a number from 4 to 8, wherein y is a number from 1 to 20, wherein z is a number from 0 to 6, and wherein n is a number from 2 to 5, said material containing between about 25 and 100 carbon atoms per molecule.

2. A lubricating composition according to claim 1 wherein R represents a branched chain alkyl group having about 8 carbon atoms, wherein X is oxygen, wherein x is 8, y is 4, z is 0, and n is 2.

30

#### References Cited in the file of this patent

#### UNITED STATES PATENTS

|              |                   |       |               |
|--------------|-------------------|-------|---------------|
| 2,260,295    | Carruthers        | ----- | Oct. 28, 1941 |
| 2,271,856    | Cummings          | ----- | Feb. 3, 1942  |
| 2,379,251    | Muskat et al.     | ----- | June 26, 1945 |
| 2,559,510    | Mikeska et al.    | ----- | July 3, 1951  |
| 2,573,701    | Filachione et al. | ----- | Nov. 6, 1951  |
| 2,608,577    | Weesner           | ----- | Aug. 26, 1952 |
| 40 2,706,534 | Hunter            | ----- | Apr. 19, 1955 |